# EUROPEAN PATENT SPECIFICATION

(11) **EP 3 380 594 B1**
(45) Date of publication and mention of the grant of the patent: **06.10.2021**
(21) Application number: 16800935.5
(22) Date of filing: 22.11.2016
(51) Int. Cl.: C10M 145/14, C10M 169/04, C10M 177/00, C10N 20/02, C10N 20/04, C10N 30/00, C10N 30/18, C10N 40/08, C10N 70/00

(54) **USE OF AN ADDITIVE FOR IMPROVING THE AIR RELEASE OF A LUBRICATING OIL**
VERWENDUNG EINES ADDITIVS ZUR VERBESSERUNG DER LUFTFREISETZUNG EINES SCHMIERÖLS
UTILISATION D'UN ADDITIF POUR AMÉLIORER LA LIBÉRATION D'AIR D'UNE HUILE LUBRIFIANTE

(30) Priority: 24.11.2015 US 201562259169 P
(43) Date of publication of application: 03.10.2018
(73) Proprietor: Shell Internationale Research Maatschappij B.V., 2596 HR The Hague (NL)
(72) Inventor: GULLAPALLI, Sravani, Houston Texas 77056 (US)
(74) Representative: Shell Legal Services IP
(86) International application number: PCT/EP2016/078463
(87) International publication number: WO 2017/089354

(56) References cited:
- US-A- 5 766 513
- US-A1- 2004 018 250
- US-A1- 2006 240 999
- US-A1- 2008 242 568
- US-A1- 2014 206 584

## Description

### Field of the Invention

The invention relates to the use of an additive for improving the air release of a lubricating oil.

### Background of the Invention

Lubricating oils are used to protect and lubricate surfaces in contact, and may also be used to transmit power. It is known that air entrainment can reduce the efficacy of lubricating oils. Air entrainment is a phenomenon wherein air bubbles (typically having a diameter of less than 1mm) are dispersed throughout the lubricating oil. Entrained air can be distinguished from free air (a pocket of air trapped in part of the system), from dissolved air (lubricating oils may contain between 6 and 12 percent by volume of dissolved air) and from foam (air bubbles typically greater than 1mm in diameter that congregate on the surface of the oil). Air entrainment can have a number of negative consequences including loss of lubricity, possible oxidation of the lubricating oil, noisy operation, lower efficiency and higher oil temperatures.

The air entrainment properties of a lubricating oil are typically measured using the ASTM D3427 air release test. This test measures the time needed for air entrained in the oil to reduce in volume to 0.2% under the test conditions and at the specified temperature. US5766513 discloses a method for reducing foaming of a hydrocarbon oil at both low and high temperatures and without degrading the air release time to the extent that would occur with a silicone antifoamant which comprises adding a minor amount of a combination fluorosilicone antifoamant and a polyacrylate antifoamant to said oil.

The present inventors have sought to improve the air entrainment properties of lubricating oils.

### Summary of the Invention

Accordingly, the invention provides the use of an additive wherein the additive is an alkyl acrylate polymer, mixed into a lubricating oil using a high shear mixer, for improving the air release of a lubricating oil as measured by ASTM D3427.

Such alkyl acrylate polymers have been previously used as anti-foam additives. Air release times are typically considered to get worse with the addition of additives, especially anti-foams such as silicone oils. This is explained by Duncanson in "Properties on Foam in Lubricating Oils", pages 9-13, May 2003 Lubrication Engineering, Journal of the Society of Tribologists and Lubrication Engineers.

It is surprising that incorporating the alkyl acrylate polymer into the lubricating oil with a high shear mixer affects the air release properties of the lubricating oil. With the present invention the skilled person can use the alkyl acrylate polymer to improve the air release of a lubricating oil.

### Detailed Description of the Invention

The present invention provides the use of an additive for improving the air release of a lubricating oil as measured by ASTM D3427. In the test, compressed air is blown through the lubricating oil, which has been heated to a temperature of 50°C. After the air flow is stopped, the time required for the air entrained in the oil to reduce in volume to 0.2% is recorded as the air release time. A desirable air release value is typically less than 3 minutes, preferably less than 60 seconds and most preferably less than 20 seconds.

The air release is improved as compared to air release achieved using the lubricating oil wherein the additive has not been mixed with the lubricating oil using a high shear mixer. The inventors have found useful reductions in air release times when carrying out the method of the invention.

The lubricating oil comprises a base oil component, which may be a blend of several base oils. The base oils in the base oil component may be any conventional base oils chosen from Groups I, II, III, IV or V of the API (American Petroleum Institute) base oil categories. Preferably the base oil component comprises a GTL base oil, and more preferably the base oil component comprises at least 75wt% of a GTL base oil based upon the weight of the base oil component. GTL base oils are synthesised by the Fischer-Tropsch method of converting natural gas to liquid fuel. They have a very low sulphur content and aromatic content compared with mineral oil base oils refined from crude oil and have a very high paraffin constituent ratio.

The lubricating oil suitably comprises additives. Preferably the amount of additives is less than 10wt% based upon the weight of the lubricating oil, more preferably less than 5wt%, most preferably less than 2.5wt%. The additives may include antioxidants, antiwear additives, demulsifiers, emulsifiers, rust and corrosion inhibitors, VI improvers and/or friction modifiers.

Preferably, the lubricating oil has a kinematic viscosity in the range of from 5 to 220cSt at 40°C, more preferably of from 10 to 200cSt, most preferably of from 20 to 100cSt. The kinematic viscosity is suitably measured using ASTM D445 (ASTM D7042).

In a preferred embodiment of the invention, the lubricating oil is formulated for use a hydraulic fluid. Hydraulic fluids are used in many different types of hydraulic machinery and are used not only to lubricate the machinery but also to transmit pressure. Air entrainment can be a particular issue in hydraulic systems, causing spongy or erratic operation of the hydraulics.

In the use according to the invention an alkyl acrylate polymer additive is mixed into the lubricating oil. Suitable alkyl acrylate polymers are disclosed in, for example, US3166508. The molecular weight of the polymer is suitably less than 10,000, preferably less than 7,500 and more preferably less than 5,000. In one embodiment the alkyl acrylate polymer may be a homopolymer of an alkyl acrylate having at least 3 but less than 7 carbon atoms in the alkyl radical. In another embodiment the alkyl acrylate polymer may be a copolymer of at least two different alkyl acrylates in which the alkyl radical has from 1 to 18 carbon atoms and in which the average number of carbon atoms in the alkyl radicals of the copolymer molecular is at least 3 but less than 7 on a molar basis.

Suitably at least 0.0005wt% of alkyl acrylate polymer, based upon the weight of the lubricating oil, is mixed into the lubricating oil, preferably at least 0.001wt%. Suitably less than 0.1wt% of alkyl acrylate polymer, based upon the weight of the lubricating oil, is mixed into the lubricating oil, preferably less than 0.01wt%. The preferred amount of alkyl acrylate polymer will be a balance between using enough to achieve the desired improvement in air release properties and avoiding unnecessary expense by using too much alkyl acrylate polymer.

The alkyl acrylate polymer additive is mixed into the lubricating oil using a high shear mixer. The term "high shear mixer" is well-known to persons skilled in the art. A rotating impeller or high-speed rotor creates flow and shear within the liquid that is mixed. In some embodiments the rotor will turn within a stationary component known as a stator. Preferably the additive is mixed into the lubricating oil at a rate of at least 400rpm. The rate is preferably at least 600rpm and more preferably at least 800rpm. Preferably the mixing is for at least 10 minutes, more preferably at least 30 minutes, and most preferably at least 60 minutes.

The invention is further explained in detail below by means of examples, but the invention is in no way limited by these examples.

### Examples

Seven different base oil blends were prepared using combinations of three base oils:
1) Chevron 220 R (a Group II mineral oil available from Chevron)
2) XHVI 8 (a Fischer-Tropsch derived oil available from Shell)
3) Spectrasyn 8 (a poly-alpha olefin fluid available from ExxonMobil)

Table 1 gives the amounts of each base oil (in weight % based upon the total weight of the blend) present in each blend. The blends in Table 1 are all ISO 46.

**Table 1**

| | Chevron 220 R | XHVI 8 | Spectrasyn 8 |
|---|---|---|---|
| Blend 1 | 15 | 80 | 5 |
| Blend 2 | 25 | 70 | 5 |
| Blend 3 | 15 | 75 | 10 |
| Blend 4 | 20.0 | 72.5 | 7.5 |
| Blend 5 | 20 | 80 | 0 |
| Blend 6 | 25 | 75 | 0 |
| Blend 7 | 0 | 100 | 0 |

An additive package containing extreme pressure/antiwear additive, friction modifier, ashless rust inhibitor, emulsifier and antioxidant was added to the base oil blends to provide fully formulated lubricating oils. The additive package was the same in each instance. Then 125 ppm of PC 3144 additive (available from Allnex), which is a 40% solution of a modified acrylic polymer in a hydrocarbon solvent, was added to the formulations at 40°C either at a stirring rate of 1200rpm using an overhead Caframo high shear mixer for an hour or at a stirring rate of 300rpm using a magnetic stirrer for an hour.

The air release time of the base oil blends, of the fully formulated oils and of the fully formulated oils plus PC 3144 was tested using the ASTM D3427 method. The results are given in Table 2:

**Table 2**

| | Air release time at 50°C (seconds) | | | |
|---|---|---|---|---|
| | Base oil blend | Fully formulated oil | Fully formulated oil plus PC 3144 with high shear mixer | Fully formulated oil plus PC 3144 with magnetic stirrer |
| Blend 1 | 5 | 16 | 5 | Not measured |
| Blend 2 | 31 | 31 | 5 | Not measured |
| Blend 3 | 5 | 5 | 5 | Not measured |
| Blend 4 | 20 | 26 | 5 | Not measured |
| Blend 5 | 5 | 31 | 16 | 10 |
| Blend 6 | 15 | 10 | 5 | 19.8 |
| Blend 7 | 5 | 5 | 5 | 10 |

The results show that air release of the base oil blends varies. Adding the additive package can further increase the air release time. Adding the PC 3144 additive using a high shear mixer can substantially reduce the air release time (unless the air release time is already very low as was the case for Blend 3 and Blend 7). Adding the PC 3144 additive with a magnetic stirrer does not seem to have the same effect.

## Claims

1. The use of an additive, wherein the additive is an alkyl acrylate polymer, mixed into a lubricating oil using a high shear mixer, for improving the air release of the lubricating oil as measured by ASTM D3427.

2. A use according to claim 1, wherein the lubricating oil comprises a base oil component, and the base oil component comprises at least 75wt% of a GTL base oil based upon the weight of the base oil component.

3. A use according to claim 1 or claim 2, wherein the lubricating oil has a kinematic viscosity in the range of from 5 to 220cSt at 40°C.

4. A use according to any preceding claim, wherein the lubricating oil is formulated for use a hydraulic fluid.

5. A use according to any preceding claim, wherein the molecular weight of the alkyl acrylate polymer is less than 10,000.

6. A use according to any preceding claim, wherein the alkyl acrylate polymer is a homopolymer of an alkyl acrylate having at least 3 but less than 7 carbon atoms in the alkyl radical, or the alkyl acrylate polymer is a copolymer of at least two different alkyl acrylates in which the alkyl radical has from 1 to 18 carbon atoms and in which the average number of carbon atoms in the alkyl radicals of the copolymer molecular is at least 3 but less than 7 on a molar basis.

7. A use according to any preceding claim, wherein at least 0.0005wt% and less than 0.1wt% of alkyl acrylate polymer, based upon the weight of the lubricating oil, is mixed into the lubricating oil.

8. A use according to any preceding claim, wherein the additive is mixed into the lubricating oil at a rate of at least 400rpm.

9. A use according to any preceding claim, wherein the additive is mixed into the lubricating oil at a rate of at least 800rpm.

## Patentansprüche

1. Verwendung eines Additivs, wobei das Additiv ein Alkylacrylatpolymer ist, das unter Verwendung eines Mischers mit hoher Scherung in ein Schmieröl zum Verbessern der Luftabscheidung des Schmieröls eingemischt wird, gemessen durch ASTM D3427.

2. Verwendung nach Anspruch 1, wobei das Schmieröl eine Basisölkomponente umfasst und die Basisölkomponente wenigstens 75 Gew.-% eines GTL-Basisöls, basierend auf dem Gewicht der Basisölkomponente, umfasst.

3. Verwendung nach Anspruch 1 oder 2, wobei das Schmieröl eine kinematische Viskosität in dem Bereich von 5 bis 220 cSt bei 40 °C aufweist.

4. Verwendung nach einem der vorhergehenden Ansprüche, wobei das Schmieröl zur Verwendung als ein Hydraulikfluid formuliert ist.

5. Verwendung nach einem der vorhergehenden Ansprüche, wobei die Molekularmasse des Alkylacrylatpolymers weniger als 10.000 beträgt.

6. Verwendung nach einem der vorhergehenden Ansprüche, wobei das Alkylacrylatpolymer ein Homopolymer eines Alkylacrylats ist, das wenigstens 3, jedoch weniger als 7 Kohlenstoffatome in dem Alkylrest aufweist, oder das Alkylacrylatpolymer ein Copolymer von wenigstens zwei verschiedenen Alkylacrylaten ist, in dem der Alkylrest von 1 bis 18 Kohlenstoffatome aufweist und in dem die durchschnittliche Anzahl von Kohlenstoffatomen in den Alkylresten des Copolymermoleküls wenigstens 3, jedoch weniger als 7 auf einer molaren Basis beträgt.

7. Verwendung nach einem der vorhergehenden Ansprüche, wobei wenigstens 0,0005 Gew.-% und weniger als 0,1 Gew.-% Alkylacrylatpolymer, basierend auf dem Gewicht des Schmieröls, in das Schmieröl eingemischt werden.

8. Verwendung nach einem der vorhergehenden Ansprüche, wobei das Additiv mit einer Rate von wenigstens 400 U/min in das Schmieröl eingemischt wird.

9. Verwendung nach einem der vorhergehenden Ansprüche, wobei das Additiv mit einer Rate von wenigstens 800 U/min in das Schmieröl eingemischt wird.

## Revendications

1. Utilisation d'un additif, dans laquelle l'additif est un polymère d'acrylate d'alkyle, mélangé à une huile lubrifiante à l'aide d'un mélangeur à cisaillement élevé, afin d'améliorer la libération d'air de l'huile lubrifiante telle que mesurée par la norme ASTM D3427.

2. Utilisation selon la revendication 1, dans laquelle l'huile lubrifiante comprend un composant d'huile de base, et le composant d'huile de base comprend au moins 75 % en poids d'une huile de base GTL par rapport au poids du composant d'huile de base.

3. Utilisation selon la revendication 1 ou la revendication 2, dans laquelle l'huile lubrifiante a une viscosité cinématique dans la plage de 5 à 220 cSt à 40 °C.

4. Utilisation selon l'une quelconque des revendications précédentes, dans laquelle l'huile lubrifiante est formulée pour être utilisée comme fluide hydraulique.

5. Utilisation selon l'une quelconque des revendications précédentes, dans laquelle le poids moléculaire du polymère d'acrylate d'alkyle est inférieur à 10 000.

6. Utilisation selon l'une quelconque des revendications précédentes, dans laquelle le polymère d'acrylate d'alkyle est un homopolymère d'un acrylate d'alkyle ayant au moins 3 mais moins de 7 atomes de carbone dans le radical alkyle, ou le polymère d'acrylate d'alkyle est un copolymère d'au moins deux acrylates d'alkyle différents dans lequel le radical alkyle a de 1 à 18 atomes de carbone et dans lequel le nombre moyen d'atomes de carbone dans les radicaux alkyle du copolymère moléculaire est d'au moins 3 mais moins de 7 sur une base molaire.

7. Utilisation selon l'une quelconque des revendications précédentes, dans laquelle au moins 0,0005 % en poids et moins de 0,1 % en poids de polymère d'acrylate d'alkyle, par rapport au poids de l'huile lubrifiante, est mélangé dans l'huile lubrifiante.

8. Utilisation selon l'une quelconque des revendications précédentes, dans laquelle l'additif est mélangé dans l'huile lubrifiante à une vitesse d'au moins 400 tr/min.

9. Utilisation selon l'une quelconque des revendications précédentes, dans laquelle l'additif est mélangé dans l'huile lubrifiante à une vitesse d'au moins 800 tr/min.
